

## UNITED STATES PATENT OFFICE

MAX BAER, OF NEW YORK, N. Y.

## INK PRODUCT AND PROCESS OF MAKING THE SAME

No Drawing.

Application filed August 8, 1929. Serial No. 384,487.

The present invention relates to an ink product and process of making the same, the invention being more particularly related to an improved printing ink product and its process of manufacture.

Hitherto, in the art of lithographing, label printing and in similar lines of work, it has been the practice to print gold size on the sheets, allow the printing to dry to a certain extent and become "tacky", and then to print thereon gold or other colored bronzes. Under this practice it has been customary to carry out two distinct printing operations; first, the printing of the gold size, and then the printing of the gold bronze. In addition to these two distinct operations, there is another attendant disadvantage in that the gold bronze which is printed in dry powdered form escapes into the surrounding atmosphere and thence settles upon the printing machines, paper stock and persons within the printing room, the powdered gold bronze frequently having an injurious effect upon the persons inhaling the same.

The object and purpose of my invention are to provide a ready mixed gold or other colored bronze, having the character of an ink, either in liquid, semi-liquid or paste form, capable of being applied in one printing operation.

Another object is to provide an improved product, as stated, whereby lithographers, label printers and others engaged in printing sheets in gold bronzes may perform their work quickly, economically, and without the use of the powdered product.

Other objects will appear hereinafter.

My improved product consists of a mixture of cresylic acid, sulphuric acid, borax, flour, chrome yellow and gold bronze, together with a vehicle which holds the other elements in a suitable ready mixed state until they have been printed upon the sheet.

The best formula embodying my invention at present known to me, and the preferred process of making, compounding and using the same, according to my present information, is as follows:

I make a product aggregate consisting, by weight, of about thirty percentum of the

base ingredients, commercially referred to as pigments, and seventy percentum of vehicle materials, although these proportions may be varied greatly in accordance with the general character of the product to be obtained, whether in the form of a thin liquid paste ink, a semi-paste ink or a full paste ink. For the base or pigment aggregate, entering into the product, I prefer to use ingredients in about the following proportions, by weight, cresylic acid eight percentum, sulphuric acid four percentum, borax fifteen percentum, flour sixty percentum, chrome yellow three percentum and gold bronze ten percentum. For the vehicle aggregate, entering into the product, I prefer to take about ninety percentum of water and ten percentum of varnish. Good results may be obtained, however, when the materials, both of the pigments and vehicles, are varied within the limits of twenty percentum of the proportions given.

All of the materials may be introduced and mixed at the same time, and they are cooked at about boiling temperature until thoroughly and uniformly mixed as a ready mixed product in the state desired, that is to say, a thin liquid paste ink, a semi-paste ink or a full paste ink.

The improved ink product produced as above described is very economical in manufacture, and is highly efficient as a ready mixed gold ink or bronze ink.

The method of application may vary in accordance with the character of the printing press, device or apparatus used in printing. It is, of course, well known that lithographers use either an offset printing machine or a flat-bed litho press. When employing the offset machine the lithographers print from an aluminum or zinc plate. Where a flat-bed press is used the printing is done from a stone. Label printers print from an electro-plate. My ready mixed ink product can be used to advantage in all of these methods of printing. In press printing the especially prepared plate is very sensitive to grease. When the press is set in motion a set of flannel rollers (kept moist by contact with water) pass over the surface of the plate, slight-

ly wetting it. Immediately following the damp rollers are the ink rollers, which distribute the ready mixed ink product smoothly and evenly over the designs on the surface of the plate. In this process, the thin coating of water prevents the ink product from adhering to the plate and only the designs thereof receive an application of the ink product.

- 10 It may be remarked here that whenever the ready mixed gold or bronze ink product is too heavy, the same may be reduced to a suitable consistency by the addition of a suitable grease compound, for instance, petroleum jelly or varnish. In this way, the consistency of the product may be varied according to the character of the work and according to the judgment of the man in charge of the press.
- 15 20 While I have given above the best formula embodying my invention at present known to me, and the preferred process of making, compounding and using the same, I realize that in practice other combinations of pigments might be used besides those before mentioned, and the process of compounding may be varied as experience dictates, to produce the precise character and color of ready mixed gold or other colored bronzes as may be desired for printing purposes. It is to be understood, therefore, that changes and modifications in the formula and in the process of making the product may be made therein, to which changes and modifications I am entitled, provided the same are effected within the scope of the annexed claims.

Having now particularly described and ascertained the nature of my said invention and in what manner the same is to be performed, I declare that what I claim is:

1. The herein described ink product adapted for use by lithographers, label and other printers, as a ready mixed product, characterized by including as pigments chrome yellow and gold bronze in the presence of a mixture containing sulphuric acid, cresylic acid and borax.
2. The herein described ink product adapt-

ed for use as a ready mixed printing ink, characterized by including sulphuric acid, borax, flour, chrome yellow and gold bronze, and a vehicle with water and varnish for retaining the elements in a state for even distribution.

3. The herein described ink product adapted for use as a ready mixed printing ink, characterized by including cresylic, sulphuric acid, borax, flour, chrome yellow and gold bronze, with a preponderating quantity of vehicle comprising water and varnish.

4. The herein described ink product adapted for use as a ready mixed printing ink, characterized by including three parts pigment and seven parts vehicle, the pigment consisting of eight parts cresylic, four parts sulphuric acid, fifteen parts borax, sixty parts flour, three parts chrome yellow and ten parts gold bronze, and the vehicle consisting of ninety-two to ninety-five parts water and five to ten parts varnish.

5. The herein described process of producing a ready mixed printing ink product, which consists in mixing cresylic, sulphuric acid, borax, flour, chrome yellow and gold bronze with a preponderating quantity of water and varnish, and cooking the mixture to produce a thin paste form, a semi-paste form or full paste form, as desired.

6. The herein described process of producing a ready mixed printing ink product, consisting in mixing in water and varnish, cresylic, sulphuric acid, borax, flour and a pigment, and in subjecting the mixture to the action of heat to produce the desired ready mixed consistency.

7. The process of making a ready mixed printing ink, which consists in mixing 30% by weight of base ingredients and 70% by weight of vehicle materials and then boiling the resultant mixture to obtain a uniform mixture, said base ingredients including cresylic acid, sulphuric acid, borax, flour, chrome yellow and gold bronze, and vehicle materials containing water and varnish.

MAX BAER.

50

55

60

65

115

120

125

130